

## UNITED STATES PATENT OFFICE

GEORG PEMETZRIEDER, OF BERLIN-TEMPELHOF, GERMANY

## ALLOY WITH COPPER AS PRIMARY METAL

No Drawing. Application filed May 1, 1931, Serial No. 534,449, and in Germany May 2, 1930.

Many attempts have been made to produce lead alloys especially adapted for bearing metal by adding other materials to lead. Such an alloy must answer the physical and mechanical requirements demanded by this use in the highest possible degree; that is to say, it must have sufficient hardness, good plasticity, high compressive strength, and favorable gliding qualities.

- 10 In German Patents 420,068 and 423,292 this method, consisting in refining lead by addition of other materials, is departed from, and instead, expensive alloys, such as bronze, are spread or diluted by the addition of lead.
- 15 At the same time there are added to the copper and tin, in addition to a maximum of about 25% of lead, small percentages of nickel and zinc. In German Patent 436,440 bronze is again the base metal and, beside 20 lead and tin, zinc, vanadium, and refractory metals are added to improve the alloy.

The essential novel idea of the present invention which distinguishes it from the prior art is the spreading of an alloy having copper as a base metal by the addition of lead refined by the addition of alkali metals.

Heretofore tin-bronzes with proportions of lead varying within wide limits have been found to be adapted for many different purposes. The usefulness of these bronzes is greatly increased by raising their lead content with the accompanying increase in plasticity, on the other hand the proportion of lead which can be added is influenced to a great extent by its qualities. The lead added to the bronze base alloy is only taken up in solid solution to a slight degree. Most of the lead separates in the form of small drops and thereby becomes a determining factor of the alloy.

Pure lead has very little hardness (Brinell hardness about 3.6 to 3.8 kg. per sq. mm.) and is for this reason not well adapted for bearing metal, for example. It has a tendency to smear, due to its very low strength, and is therefore the frequent cause of failures of full leaded axle boxes of bronze alloys having a high proportion of lead. For this reason, up to this time an admixture of 15

to 20% lead in the alloy has been found to be the optimum limit.

According to the present invention instead of pure lead there are used hardened lead alloys, which practice has shown to be 55 exceptionally good for bearing purposes, for example. These hardened lead alloys (Brinell hardness 30-45 kg. per sq. mm.) can be very easily produced from pure lead by the addition of alkali or alkaline earth metals, 60 and can be brought into the alloys having copper as a base metal without difficulty. These base alloys may consist of pure copper-tin, or may have zinc as an added metal. The alkali metal content causes a good dispersion of the hardened lead alloy in the bronze and the troublesome liquation is considerably repressed. This is an important technical improvement in alloys. Experiments have shown that in such an alloy 70 increased hardness, superior compressive strength with good plasticity, and, when used as bearing metal, for example, very favorable gliding qualities are attained.

In the following tables a lead bronze as 75 previously used and one composed in accordance with the invention are compared:

| Lead bronze                                                                                                | Bronze according to the invention                        | 80 |
|------------------------------------------------------------------------------------------------------------|----------------------------------------------------------|----|
| 70.0% Cu<br>5.0% Sn<br>25.0% Pb                                                                            | 70.0% Cu<br>5.0% Sn<br>24.64% Pb<br>0.16% Ca<br>0.20% Na | 65 |
| Brinell hardness 49-50 kg. per sq. cm.<br>Effective compressive strength 2750 kg. per sq. cm.<br>Reduction | 58-60 kg. per sq. cm.<br>3450 kg. per sq. cm.<br>45%     | 70 |

Tests of alloys in accordance with the invention have shown that its wear is particularly low and the troublesome smearing which occurs with previously used alloys is prevented.

According to the invention a certain percentage of zinc also may be added to the primary alloy. In the following table there is given another comparison of an alloy used heretofore and one in accordance with the invention.

| Lead bronze                                   | Bronze according to the invention                                                             |
|-----------------------------------------------|-----------------------------------------------------------------------------------------------|
| 63-47% Cu<br>4-8% Sn<br>3-10% Zn<br>30-35% Pb | 62.8-46.2% Cu<br>4-8% Sn<br>3-10% Zn<br>30-35% Pb<br>0.10-0.5% alkaline earth<br>0.10-0.3% Na |

The alloy according to the invention is distinguished further by a greater mechanical solidity.

A small percentage of nickel can be added also to the alloy to obtain greater homogeneity.

15 The alloy can be made up by adding the hardened lead alloy to the base alloy in solid or liquid state with simultaneous thorough mixing, or it can be made by mixing all the alloying elements together in the manner described.

20 Having described my invention, I claim:  
1. An alloy composed of the following ingredients in approximately the proportions given: copper 62.3% to 46.2%, tin 4 to 8%, zinc 3 to 10%, lead 30 to 35%, alkaline earth metal 0.2 to 0.5%, and sodium 0.1 to 0.3%.

25 2. A lead bronze alloy containing about 4 to 8% of tin, about 3 to 10% zinc, about 20 to 35% of lead, about 0.1 to 1% of one or more metals selected from the alkali and alkaline earth group, the remainder principally copper.

30 3. A bearing composed of the alloy described in claim 2.

35 4. A lead bronze alloy containing about 5% of tin, 3 to 10% of zinc, about 24.5% of lead, about 0.1 to 0.2% of one or more metals selected from the alkali and alkaline earth group, the remainder principally copper.

40 5. A bearing composed of the alloy described in claim 4.

45 6. A lead bronze alloy having the composition stated in claim 2 and containing in addition a small percentage of nickel to improve the homogeneity.

7. A bearing composed of a lead bronze alloy having the composition stated in claim 2 and containing in addition a small percentage of nickel to produce greater homogeneity.

50 In testimony where I affix my signature.

GEORG PEMETZRIEDER.